

# UNITED STATES PATENT OFFICE.

EDWIN JAMES LOVEGROVE AND NIGEL GEORGE CROMPTON, OF LONDON, ENGLAND;  
ELIZABETH GERTRUDE CROMPTON EXECUTRIX OF SAID NIGEL GEORGE CROMPTON,  
DECEASED; SAID EXECUTRIX ASSIGNEE TO SAID LOVEGROVE.

## BITUMINOUS GROUTING.

1,237,921.

Specification of Letters Patent. Patented Aug. 21, 1917.

No Drawing.

Application filed March 2, 1915. Serial No. 11,582.

To all whom it may concern:

Be it known that we, EDWIN JAMES LOVEGROVE and NIGEL GEORGE CROMPTON, subjects of the King of England, both residing in London, England, have invented certain new and useful Improvements in Bituminous Grouting, of which the following is a specification.

This invention relates to materials employed in road-making, road-dressing and the like and refers particularly to a bituminous grouting as distinct from a paving material, that is to say as distinct from a material which of itself alone will constitute a traffic-resisting surface.

In the preparation, for instance, of Macadam roads and roads formed of granite sets or wood-blocks, the interstices are wholly or partly grouted or filled with fluid composition which will set comparatively hard. Hitherto bituminous groutings have been composed of bitumen and a gritty filler such as sand or other finely-divided manufactured or mineral matter. Also a grouting has previously been proposed consisting of approximately equal proportions of purified tar or pitch and retorted shale or residue or ash of shale that has been treated in a retort or the like or calcined coal or the residue due or ash of coal reduced to a fine impalpable powder.

According to the present invention the grouting is composed of bituminous material combined with a filler composed of clinker or ash or like residue of combustion in a fine impalpable condition and preferably obtained from a refuse- or dust-destructor. The bituminous material employed is either bitumen produced by the evaporation of asphaltic oils, or natural or native bitumen.

Throughout the specification and claims whenever the term "refuse destructor residue" is employed, it is to be understood as indicating all forms of vitrified clinker or ash or like residue of combustion from a refuse destructor or incinerator, other than coal or coke clinker or ash.

Broadly speaking, the percentage of bituminous material will vary from 30-70% by weight of the whole and the proportion of finely ground clinker will be from 70-30% by weight respectively. It is preferred,

however, to employ about 50% of each ingredient although it will be understood that the proportions must vary widely with the quality and grading of the filling material and with the nature of the bituminous material employed.

The temperature at which the ingredients are mixed is that generally employed in the preparation of bituminous grouting and in general terms is that at which the bituminous material is in a sufficiently fluid condition to permit the filler to become thoroughly and evenly incorporated in it.

The powdered filling material must be in a very fine state of sub-division as otherwise a homogeneous mixture of the bituminous material and the filler cannot be maintained while the material is being handled. Preferably as the clinker or the like is being ground a very fine dust is produced which ordinarily will not be collected with the ground material, but for the purposes of the present invention this fine dust is collected during the crushing operation by means of a fan or other suction or exhaust apparatus suitably disposed in relation to the crushing device, or it may be collected subsequently to the crushing operation. It is found that the fine powder thus collected is most suitable for the present invention.

The grouting may be poured over the road-surface in the ordinary manner or by flowing it on to the surface and finally distributing it with a broom, squeegee or the like, or may be forced into the road-surface under pressure.

It is found that a grouting prepared with bituminous material according to the present invention has many advantages over the grouting prepared with tar or pitch and among these advantages may be mentioned the following:

Tar or pitch grouting, at ordinary temperatures, has a tendency to flow and it is mainly plastic as distinct from a mainly elastic property possessed by the bituminous grouting according to the present invention. Also a tar or pitch grouting is liable to perish and to become absorbent owing to evaporation of oils originally contained in the tar or pitch. On the contrary a bituminous grouting according to this invention does not perish or deteriorate in this manner and

is, for all practical purposes, at all times non-absorbent.

What we claim as our invention and desire to secure by Letters Patent is:—

- 5 1. A grouting or binder composed of refuse destructor residue in the form of a fine powder combined with bituminous material.
2. A grouting or binder composed of a refuse destructor residue in the form of a fine powder combined with bituminous material.
- 10 3. A grouting or binder composed of a refuse destructor residue in the form of a fine powder combined with bituminous material in the proportions by weight of 75 per cent. to 60 per cent. of residue with 25 per cent. to 40 per cent. of bituminous material.
3. A grouting or binder composed of ref-

use destructor residue in the form of a fine powder combined with bituminous material in the proportions by weight of 70 per cent. of residue to 30 per cent. of bituminous material.

In testimony whereof we have signed our names to this specification in the presence of two subscribing witnesses.

EDWIN JAMES LOVEGROVE.  
NIGEL GEORGE CROMPTON.

Witnesses:

HAROLD WADES,  
HARRY K. WISELY.